

W. B. D. PENNIMAN AND R. S. WHITE,  
PRODUCTION OF FERROSILICON ALUMINUM,  
APPLICATION FILED JUNE 9, 1919.

1,369,298.

Patented Feb. 22, 1921.



William B. D. Penniman, Inventor.  
Ray S. White

WITNESSES.

Frank R. Edwards

Mary C. Miller.

By Edward F. Daniels

Attorney

# UNITED STATES PATENT OFFICE.

WILLIAM B. D. PENNIMAN AND ROY S. WHITE, OF BALTIMORE, MARYLAND.

## PRODUCTION OF FERROSILICON ALUMINUM.

1,369,298.

Specification of Letters Patent. Patented Feb. 22, 1921.

Application filed June 9, 1919. Serial No. 302,863.

*To all whom it may concern:*

Be it known that we, WILLIAM B. D. PENNIMAN and ROY S. WHITE, citizens of the United States of America, and residents of the city of Baltimore, State of Maryland, have invented certain new and useful Improvements in the Production of Ferrosilicon Aluminum, of which the following is a specification.

10 This invention relates to the direct production on a commercial scale of a combination of aluminum, iron and silicon, known as ferro-silicon aluminum.

In the manufacture of ferro-silicon, which is used as a "scavenging or purging" agent in the production of cast iron and steel, a small amount of aluminum sometimes appears as an impurity. This is distinguished from the subject of the present disclosure, first, by the fact that this small amount of aluminum occurs as a result of what must be considered an impurity in the materials used in the manufacture of ferro-silicon, because this aluminum content in 25 the materials is a disadvantage in the manufacture of ferro-silicon as now practised, and, second, in the product, aluminum is not present in amounts sufficient to be of practical advantage to the maker of ferro-silicon or the user of it, and it is not customary to make any financial allowance for its presence or to consider it as a factor in the use of the ferro-silicon or its application to the arts.

35 The presence of these impurities containing aluminum in the materials used in the manufacture of ferro-silicon is to be avoided under ordinary conditions because they give rise to a troublesome slag which has such a high melting point that it is difficult to remove from the furnace and separate from the ferro-silicon. These impurities as they have occurred also give off an increased amount of dust, the proportion of aluminum 40 oxid found in such dust being far in excess of the proportion of aluminum oxid present in the ores and other constituents introduced into the furnace, so that the aluminum content in the materials is mostly lost 45 and only small amounts in proportion appear in the ferro-silicon.

In our experience operating with these impure materials the amount of aluminum found in ferro-silicon is generally much

less than 1% and seldom, if ever, exceeds 2%.

It is well known that an alloy or combination of aluminum, iron and silicon is on the market and is known as ferro-silicon aluminum. This combination is effected, 60 however, by making in separate and distinct operations, ferro-silicon and metallic aluminum, which are afterward melted and compounded together to form the desired product.

65 Our invention comprises a new method of making an alloy of aluminum, iron and silicon which has evident advantages so far as cost and convenience of manufacture on a large scale are concerned.

70 The product of the process which is the subject of this invention contains on an average of from 15 to 20% aluminum and is intended to include any per cent. from 3 or 4 to 50%.

75 At the present time large quantities of ferro-silicon are used as a scavenger or purging agent in the manufacture of iron and steel. It is also customary to use metallic aluminum for the same general purposes; sometimes both of them are used in the same batch of metal, ferro-silicon being used first and the aluminum afterward, as the latter is generally considered a more active agent in removing impurities and it 80 is also believed to have an effect upon certain substances that are not affected by the ferro-silicon.

85 Metallic aluminum is however used at great disadvantage, first, on account of its expense and, second, on account of the waste. The latter arises from the fact that the boiling point of the metal is low and it oxidizes so readily that only a small part of what is used is effective. It is estimated 90 that only about 10% of what is applied actually finds its way into the steel, 90% being lost in the way indicated.

95 With ferro-silicon-aluminum there is on the other hand a much more effective use of 100 aluminum as the metal is protected in a large measure from oxidation by the air and in this combination with the other constituents of the alloy, it can be introduced much more effectively into the body of 105 molten steel or iron.

It is wellknown that the production of aluminum is necessarily expensive on ac-

count of the purity of the materials required and the comparative complexity of the apparatus used. When the ferro-silicon-aluminum is made direct from ferro-silicon and aluminum, there is the high cost inherent to the production of aluminum and also the losses of aluminum that occur when the metal is combined with ferro-silicon. These losses of aluminum are not perhaps 10 as great as in the ordinary practice of steel or iron making but they are so large that the price of ferro-silicon-aluminum is high and ranges far above the cost of the ferro-silicon and aluminum purchased separately. On 15 the other hand, ferro-silicon-aluminum can be made according to this invention direct from cheap iron, silicon and aluminum compounds which occur abundantly in nature.

20 In the early development of the invention the product, *i. e.*, ferro-silicon-aluminum was produced by treating brick bats and coke in an electric furnace, such as is ordinarily used for making ferro-silicon, the 25 proportions by weight being seven of brick to nine of coke. The brick-bats and the ash of the coke are both intimate mixtures or chemical combinations of aluminum oxids, silicon and iron oxids, and similar except as to 30 the presence of small and unimportant amounts of other substances. By proper management of the furnace the desired material was obtained as indicated below.

To reduce still further the loss by way of 35 the stack and the difficulties of slag formation, we may preferably, though not necessarily, as a partial source of aluminum, use some compound of aluminum and silica that contains in addition other material or materials that act as a flux. By preference we 40 have been using commercial feldspar which is in the main potassium aluminum silicate. In practice an impure feldspar may be used or the fluxing material may be some other 45 compound. This fluxing material may be introduced as a separate substance. At the present time ordinary feldspar is the best material as it is cheap and plentiful, particularly as we do not require the high quality 50 of feldspar that is necessary for other industrial uses and can in consequence avail ourselves of what would otherwise be a waste product at the mines where feldspar is produced.

55 In the practice of the method of the invention, both the slagging and consequent loss of aluminum and dust losses by volatilization of aluminum oxids are in a large measure avoided.

60 The materials are mixed in proportions determined by the product desired and fed gradually into the furnace. It is important that the arc should be kept covered as far as possible and the electrodes well under the 65 charge. The spacing of the electrodes is

proportionate to the voltage and in accordance with regular practice in the operation of electric furnaces used in the manufacture of ferro-alloys of this general character.

An alloy containing approximately 15% 70 aluminum, 35% of silicon and the balance iron can be readily produced from the materials mentioned above. If a higher percentage of aluminum be desired, bauxite or some other compound containing a higher 75 proportionate amount of aluminum and less iron and silica can be added to the mixture or a clay or clay product, containing less iron or silicon may be used. It is also true that at times we find it advisable with the 80 materials indicated above to add either iron oxid or metallic iron or silica in the form of silica rock. These variations in materials depend upon the kind of alloy we desire to make and the market price of the different 85 ores available. By using selected materials the amount of aluminum can be carried as high as 30 to 40% or even 50%. As an example of the flexibility with which the process can be applied with a saving of cost of 90 raw materials and in this instance with a better yield, we have used the following materials to produce practically the same alloy as that indicated above:

150 pounds feldspar.

150 pounds coke.

25 pounds iron ore (90% iron oxid).

In this particular case the product contained 44.15% silica, 40.10% iron and 15.64% aluminum. It should be stated that the 100 figures given above only show proportions as our operations have been on a large scale and tons may be substituted for pounds in this formula.

In general terms the method of the invention consists in treating compounds of aluminum and silicon containing or mixed with iron compound or iron, in the presence of a reducing agent, in an electric furnace substantially as described.

In the accompanying drawing, we have illustrated an electric furnace equipped for the production of ferro-silicon aluminum, in accordance with my invention, showing the preferred arrangement of the charge in 115 relation to the electrodes. The details are not, however, essential to the invention but may be widely varied.

The figure is a transverse section on a vertical plane and so placed as to disclose the 120 electrodes in elevation.

The furnace structure, 1, as shown, is built of fire bricks, 2, or any convenient material suitable to such structures, the furnace walls being formed to inclose a cavity 125 or chamber, 3, for the charge, the bottom of the cavity being, in the form of the invention shown, coated or lined with a suitable fire-proof cement or similar plastic, 4.

The buses, 5, 6, 7, connections 8, 9, 10, 130

and electrodes, 11, 12, 13, as shown, are arranged in accordance with the three wire system. The unfused charge is indicated by reference character, 14, and the fused portion 5 by reference character, 15.

The operation of the furnace in the practice of the method of the invention, is believed to be entirely clear from the foregoing description of the method.

10 We have thus described specifically and in detail a preferred and alternative method of making ferro-silicon-aluminum with sufficient definiteness to enable those skilled in the correlated metallurgical arts to practise 15 the invention; however, these specific terms and details are used in a descriptive rather than a limiting sense, the scope of the invention being defined in the claims.

What we claim and desire to secure by 20 Letters Patent is:

1. A method of making ferro-silicon aluminum alloy which consists in treating compounds of aluminum and silicon and iron and a reducing agent in an electric furnace, 25 substantially as described.

2. A method of making a ferro-silicon aluminum alloy which consists in treating compounds of aluminum and silicon and iron and a reducing agent with a flux in 30 an electric furnace, substantially as described.

3. A method of making a ferro-silicon aluminum alloy which consists in treating compounds of silica and aluminum and iron 35 in the presence of a reducing agent in an electric furnace, the materials being thoroughly mixed, substantially as described.

4. A method of making a ferro-silicon aluminum alloy which consists in treating compounds of silicon and aluminum with 40 iron in the presence of a reducing agent in an electric furnace, the materials being thoroughly mixed and fed gradually, substantially as described.

5. A method of making a ferro-silicon 45 aluminum alloy containing three to twenty per cent. of aluminum which consists in treating compounds of silicon and aluminum with iron in the presence of a reducing agent in an electric furnace, the materials 50 being thoroughly mixed and fed gradually, and the electrodes being kept covered with the materials, substantially as described.

6. A method of making a ferro-silicon aluminum alloy containing 3 to 50% alu- 55 minum which consists in treating com- pounds of aluminum and silicon with iron in the presence of a reducing agent in an electric furnace, bauxite being added to in- crease the aluminum content, substantially 60 as described.

7. A method of making ferro-silicon alu- 65 minum alloy containing over 3% of alu- minum which consists in treating feldspar in an electric furnace in the presence of a reducing agent, the furnace mix also includ- ing iron, substantially as described.

Signed by us at Baltimore, Maryland, this 2nd day of June, 1919.

WILLIAM B. D. PENNIMAN.  
ROY S. WHITE.

Witnesses:

ALFRED C. HATCH,  
EDWIN F. SAMUELS.